

Feb. 4, 1947.

J. J. SCHAEFER

2,415,374

NONMETALLIC SPRING FOR UPHOLSTERY

Filed Oct. 20, 1943

*Fig. 1.*



*Fig. 2.*



*Fig. 3.*



*Fig. 4.*



*Fig. 5.*



INVENTOR.

JUSTUS J. SCHAEFER  
BY

H. G. Manning

ATTORNEY

## UNITED STATES PATENT OFFICE

2,415,374

## NONMETALLIC SPRING FOR UPHOLSTERY

Justus J. Schaefer, Great Barrington, Mass.

Application October 20, 1943, Serial No. 506,994

5 Claims. (Cl. 5—256)

1

This invention relates to furniture and upholstery, and more particularly to an interior coiled spring made from vulcanized fiber or other similar material which is especially adapted to be used in innerspring mattresses, spring cushions, and other upholstered furniture.

One object of this invention is to provide a coiled spring of the above nature which may be made from a sheet of highly compressed vulcanized fiber or other suitable non-metallic material by a process which comprises first cutting up said sheet into a plurality of strips of square cross section, grinding said strips into circular cross section, soaking the rods formed thereby in a cold salt water solution, twisting said rods in one direction, and finally drawing said twisted rods through a heated spring-forming die in the opposite direction.

A further object is to provide a coiled spring of vulcanized fiber composition, in which a base filler of shredded canvas has been added to said composition.

A further object is to provide a spring of the above nature, in which the final coiled rod, by reason of the twisting and coiling which it has received during the process of manufacture, will permanently maintain its original resiliency, strength, pitch, and length without unwinding during use.

A further object is to provide a spring of the above nature, in which a final coating of waterproof varnish has been applied after the spring has emerged from the forming die.

A still further object is to provide a coiled spring of the above nature, which will be simple in construction, inexpensive to manufacture, easy to install and manipulate, compact, ornamental in appearance, rustless, noiseless, non-breakable, non-conductive to electricity, unaffected by heat or cold, and very efficient and durable in use.

With these and other objects in view there have been illustrated on the accompanying drawing two forms in which the invention may conveniently be embodied in practice.

In the drawing.

Fig. 1 represents a perspective view of a sheet of highly compressed vulcanized fiber prior to being cut up into a plurality of straight strips of square cross section along the lines indicated.

Fig. 2 is a perspective view of one of the cut strips indicated in Fig. 1, which is shown at the left as square in cross section, and at the right as round in cross section after it has been reduced to a circular rod of the desired size by a grinding wheel also illustrated.

2

Fig. 3 is a sectional view of a tank containing a cold salt water solution, and showing a vulcanized fiber rod in the bottom thereof being treated by said solution.

5 Fig. 4 is a perspective view on a larger scale of a vulcanized fiber rod after the next step of twisting it counterclockwise.

Fig. 5 is a diagrammatic view showing another step in the first process of manufacturing the 10 coiled spring, which consists in passing the twisted rod shown in Fig. 4 through a heated spring-forming die in a clockwise direction, and showing the protective varnish coating which is applied to the rod after it has passed through said 15 die.

Referring now to the drawing in which like reference numerals denote corresponding parts throughout the several views, the numeral 10 indicates generally a rectangular elongated sheet 20 of highly-compressed vulcanized fiber having shredded canvas incorporated therein which is adapted to be cut into strips 11 of square cross section, as indicated by the lines 12 shown in Fig. 1. At the left of Fig. 2, one of the square 25 strips 11 is shown passing to the right (as indicated by the arrow) into engagement with a grinding wheel 13 which serves to remove the longitudinal edges from the square strip 11 for converting it into a rod 14 of circular or round cross section, as shown at the right of said figure.

The next step in the first process of producing the spring stock, is to place one of the rods 14 in an elongated tank 15 containing a cold one per cent solution of salt water 16, as shown 35 in Fig. 3, and to soak said rod in the salt water bath for about twelve hours to harden, toughen, and solidify it.

The rod 14 is then removed from the tank 15, dried, and twisted in a counter-clockwise direction to increase the stiffness strength and resiliency thereof—said twist being indicated by the helical line 17 in Fig. 4.

The twisted rod 14 will then be passed through a clockwise spring-forming die 18, (as shown 45 in Fig. 5), which is preferably heated to a high temperature, causing the rod 14 to assume an open helical coil shape 19 as indicated at the right of said figure.

The final step in the process of forming the 50 coiled spring is to apply a coating 20 of a phenolic resin varnish or other similar material to the rod 14, which will permit the spring to thereafter be bent repeatedly without injury to said coating.

55 In the present application, the term "vulcanized fiber" refers to any commercial type of this

material, which may be reddish-brown, gray, black, or any other color, and of horny consistency. This material is oil proof, quite resistant to chemical action and organic solvents. It is also ductile, non-brittle and elastic. Generally, it has a tensile strength of from 8,000 to 13,000 lbs. per square inch, and a crushing strength of from 35,000 to 45,000 lbs. per square inch. Vulcanized fiber is commonly produced by running unsized unloaded rag paper through a warm solution of zinc chloride to cause it to soften and become "plastic," winding upon a roll until the desired thickness is obtained, cutting off a sheet of material and washing until all traces of the zinc chloride are removed. The resultant sheet is then subjected to compression and hardening in a press.

While there have been disclosed in this specification several forms in which the invention may be embodied, it is to be understood that these forms are shown for the purpose of illustration only, and applicant does not desire to be limited to the specific disclosure, except as required by the following claims:

Having thus fully described the invention, what is claimed as new, and for which it is desired to secure Letters Patent, is:

1. In an upholstery spring, a helical coil of highly compressed vulcanized fiber stock, said stock being twisted throughout its length on its own axis to increase the strength, stiffness and resiliency thereof and impregnated with sodium chloride to increase the toughness thereof.

2. In an upholstery spring, a helical coil of highly compressed vulcanized fiber stock having a filler of shredded canvas incorporated therewith, the stock of said coil being twisted throughout its length on its own axis to increase the strength, stiffness, and resiliency thereof and to prevent said coil from unwinding or stretching during use.

3. In an upholstery spring, a coil of highly compressed solidified plastic fibrous vulcanized fiber composition having ductile, non-brittle, elastic properties, the stock of said coil being twisted throughout its length on its own axis to

increase the strength, stiffness and resiliency thereof.

4. In an upholstery spring, a helical coil of highly compressed vulcanized fiber, the stock of said coil being twisted throughout its length on its own axis to increase the strength, stiffness, and resiliency thereof and to prevent said coil from unwinding or stretching during use.

5. In an upholstery spring, a resilient coil of solidified hardened plastic composition of vulcanized fiber having a reinforced filler of fibrous material embedded therein, the stock of said coil being twisted throughout its length to increase the strength, stiffness, and resiliency thereof.

15 JUSTUS J. SCHAEFER.

#### REFERENCES CITED

The following references are of record in the file of this patent:

#### 20 UNITED STATES PATENTS

| Number       | Name          | Date           |
|--------------|---------------|----------------|
| 71,169       | Hayward       | Nov. 19, 1867  |
| 116,557      | Cobb          | July 4, 1871   |
| 25 2,171,095 | Orsini        | Aug. 29, 1939  |
| 50,622       | Payne         | Oct. 24, 1865  |
| 99,475       | Rhinelander   | Feb. 1, 1870   |
| 101,957      | Willard       | Apr. 12, 1870  |
| 122,001      | Eagleton      | Dec. 19, 1871  |
| 30 170,973   | Tyler         | Dec. 14, 1875  |
| 2,110,029    | Shastock      | Mar. 1, 1938   |
| 2,098,082    | Bowen, et al. | Nov. 2, 1937   |
| 2,171,890    | Precourt      | Sept. 5, 1939  |
| 2,363,826    | Yellin        | Nov. 28, 1944  |
| 35 1,824,220 | Mackey        | Sept. 22, 1931 |

#### FOREIGN PATENTS

| Number | Country | Date         |
|--------|---------|--------------|
| 37,754 | German  | Dec. 9, 1886 |

#### 40 OTHER REFERENCES

Plastics Catalog (pg. 715-716) 1943—Pub. in 1942 by Plastics Cat. Corp. N. Y.—Copy in Division 50.

45